

# United States Patent

[11] 3,615,908

[72] Inventor **Frederick David Waterfall**  
Birmingham, England  
[21] Appl. No. **722,573**  
[22] Filed **Apr. 19, 1968**  
[45] Patented **Oct. 26, 1971**  
[73] Assignee **Imperial Chemical Industries Limited**  
London, England  
[32] Priority **Apr. 28, 1967**  
[33] **Great Britain**  
[31] **19,659/67**

3,228,807 1/1966 Mitchell ..... 148/16.6 X

## FOREIGN PATENTS

1,052,668 12/1966 Great Britain ..... 148/15.5  
OTHER REFERENCES

Anslegeschrift—Germany, 1170217, May 14, 1964  
Metals Handbook, 8 th Ed., Vol. 2, 1964, pub. by ASM,  
pages 129- 132

Primary Examiner—Charles N. Lovell  
Attorney—Cushman, Darby & Cushman

[54] **HEATTREATMENT OF STEEL**  
5 Claims, No Drawings

[52] U.S. Cl. ..... 148/15.5,  
148/15  
[51] Int. Cl. ..... C23c 9/16  
[50] Field of Search ..... 148/12.1,  
15, 15.5, 16.5, 16.6, 134

[56] **References Cited**

UNITED STATES PATENTS

|           |         |               |            |
|-----------|---------|---------------|------------|
| 1,499,801 | 7/1924  | Bond .....    | 148/15.5   |
| 2,264,431 | 12/1941 | Bradley ..... | 148/15     |
| 2,339,223 | 1/1944  | Holt .....    | 148/15.5   |
| 2,927,875 | 3/1960  | Mueller ..... | 148/15.5   |
| 3,194,696 | 7/1965  | Mueller ..... | 148/15.5 X |
| 3,158,514 | 11/1964 | Saxton.....   | 148/16.6 X |

**ABSTRACT:** The present invention relates to the heat-treatment of steel. More particularly it relates to the heat-treatment of all types of iron and steel which are capable of hardening on heating to the austenitising range and then quenching, without the need to introduce additional carbon during the heating step. For the sake of simplicity these types of iron and steel will be referred to hereinafter as "steel of the class which can be hardened by heating and quenching." This class of materials comprises the plain carbon steels and cast steel of the medium- and high-carbon varieties and the alloy steels containing at least 0.25 percent by weight carbon. The present invention provides a method of heat-treating steel of this class whereby the steel is provided with a surface layer that is resistant to scuffing and wear when subjected to friction under a heavy load and the underlying core is hardened so as to be resistant to indentation.

## HEATTREATMENT OF STEEL

According to the present invention we provide a method for the heat treatment of steel of the class which can be hardened by heating and quenching, which comprises heating the steel into its austenitizing temperature range in a heating medium which is noncarburizing towards the steel, then soaking the hot steel in a molten salt bath held at a temperature in the range 700°-770° C. and containing at least 5 percent by weight and preferably at least 10 percent by weight of alkali metal cyanate calculated as NaCNO for at least 3 minutes and in any case where the temperature of the salt bath is in the range 700°-750° C. preferably for at least 5 minutes, and then rapidly cooling the steel.

The austenitizing step may be carried out in a nonoxidizing gas atmosphere or in a neutral salt bath as known in the art. Alternatively, for high-carbon steels a conventional gas carburizing atmosphere or a salt bath containing cyanide salt may be employed. Although these media are generally known as carburizing media they are essentially noncarburizing in action towards high-carbon steels.

For the second step of the method according to the invention we prefer to employ a salt bath comprising alkali metal cyanide, alkali metal cyanate, alkali metal carbonate and optionally alkali metal chloride, as described in British Pat. specification Ser. No. 1,052,668 in connection with a so-called carbonitriding process. When the cyanate content of the bath is to be maintained at the preferred minimum of 10 percent by weight or higher, this can be achieved in the manner taught in the said British Specification but since the treatment temperatures used in the present invention are in general higher than the carbonitriding temperatures taught in the said British specification the iron content of the alloy steel surfaces of the container and any electrodes in contact with the molten salt bath should not exceed 22 percent by weight and should preferably be between 10 percent and 20 percent by weight. A treatment time of about 10 minutes in this type of bath is generally most useful and we have found that this treatment creates a compound layer rich in nitrogen and carbon which can be observed at the surface of an etched microsection of the treated steel. This layer at the immediate surface of the steel varies in depth from about 0.0003 inch to 0.002 inch, depending on the cyanate content and temperature of the bath, and there may also be some penetration of nitrogen further into the steel. During this treatment the steel beneath the surface layer remains mainly or wholly in the austenitic state.

After treatment in the salt bath of the second step the steel is rapidly cooled, for instance by quenching in water, oil or any other conventional quenching medium which is suitable for hardening of the particular steel. After quenching it is found that while the underlying steel or iron is hardened, with the hardest zone near the surface, the outermost layer rich in carbon and nitrogen about 0.0003-0.002 inch thick remains unchanged and possesses a very high resistance to scuffing and wear.

An alternative procedure where the usual austenitizing temperature of the steel lies within the temperature range 750°-770° C. is to carry out the austenitizing and to apply the carbon-nitrogen compound layer in the same bath. To do this the parts are heated for austenitizing by placing them directly into the said salt bath containing at least 5 percent by weight, preferably 10 percent by weight, alkali metal cyanate calculated as NaCNO, soaked for at least 7 minutes after attaining 65 bath temperature and then quenched to harden the steel.

The combination of a hardened steel or iron and a scuffing-resistant surface renders the method of the invention very useful for application to engine valve rockers in both steel and nodular iron, to various types of transmission gears and to forming tools made from plain carbon or alloy tool steels.

For articles that have to withstand extremely severe frictional conditions in use, it is preferred to maintain at least 10 percent by weight cyanate calculated as NaCNO in the salt bath used in the second treatment step, since this confers max-

imum resistance to scuffing on the surface of the treated article. Cyanate contents in the range below 10 percent but not less than 5 percent by weight are however quite acceptable for articles working under less arduous conditions; in fact the scuffing resistance achieved with cyanate contents in this range is surprisingly high and well within many commercial requirements.

The invention is further illustrated by the following example, in which all percentages are by weight, but is not limited thereby.

## EXAMPLE 1

This example shows for purposes of comparison the results obtained with a conventional hardening treatment of a tool steel.

Pieces of 0.9 percent carbon tool steel in the shape of discs 0.4 cm. in diameter suitable for testing on an Amsler wear-testing machine were hardened in the conventional manner by heating for 10 minutes in a neutral salt bath consisting of a mixture of the chlorides of sodium and potassium at 780° C. and then quenching in water. Hardness tests showed Rockwell Hardness C65-66 on the treated discs. Two treated discs, A and B, were then submitted to a wear test on an Amsler wear-testing machine. In this test the discs were rotated in edge-to-edge contact under a load of 20 kilograms at 400 and 440 r.p.m. respectively so that at the point of contact they moved in opposite directions, and they were lubricated with SAE 30 mineral oil. The discs were removed and weighed after 1,000, 9,000 and 25,000 revolutions. The test was stopped at 25,000 revolutions since by this time the discs were badly scuffed.

The loss in weight of the discs was then as follows:

|            | Grams  |
|------------|--------|
| Disc A     | 1.2623 |
| Disc B     | 0.1122 |
| Total Loss | 1.3745 |

## EXAMPLE 2

0.4 cm. diameter Amsler wear test discs made in 0.9 percent carbon tool steel, as used in example 1, were treated according to the method of the invention as follows. The discs were austenitized by heating for 10 minutes at 800° C. in a neutral salt bath consisting of a mixture of the chlorides of sodium and potassium and were then transferred directly to a salt bath maintained at 730° C. and containing 26.1 percent NaCN and 13.7 percent NaCNO, the balance being alkali metal carbonate. The discs were held in this bath for 10 minutes and were then quenched in water.

Examination of the treated discs showed the following hardness characteristics:

|                   |                            |         |
|-------------------|----------------------------|---------|
| Vickers Hardness  | HV <sub>2\frac{1}{2}</sub> | 445-463 |
| Vickers Hardness  | HV30                       | 413-418 |
| Rockwell Hardness | RHC                        | 38-40   |

Two treated discs, A and B, were submitted to a wear test on an Amsler machine as in example 1. The discs were removed at intervals and weighed. They showed no scuffing when the test was finally stopped after a total of one million revolutions. The loss in weight of the discs was then:

|            | Grams  |
|------------|--------|
| Disc A     | 0.0056 |
| Disc B     | 0.0048 |
| Total Loss | 0.0104 |

## EXAMPLE 3

0.4 cm. diameter Amsler wear test discs made in 0.9 percent carbon tool steel were austenitized by heating for 10 minutes in a neutral salt bath at 800° C. as in example 2. They were then transferred directly to a salt bath maintained at 750° C. and containing 23.0 percent NaCN and 11.3 percent NaCNO, the balance being alkali metal carbonate. The discs were held in this bath for 10 minutes and were then quenched in water.

Examination of the treated discs showed the following hardness characteristics:

|                   |      |         |
|-------------------|------|---------|
| Vickers Hardness  | HV2½ | 445-454 |
| Vickers Hardness  | HV30 | 680-690 |
| Rockwell Hardness | HRC  | 61-63   |

Two treated discs, A and B, submitted to wear testing on an Amsler machine as in example 2 showed no scuffing after a total of one million revolutions and the loss in weight of the discs during the test was as follows:

|            | Grams  |
|------------|--------|
| Disc A     | 0.3256 |
| Disc B     | 0.2430 |
| Total Loss | 0.5686 |

15

5. A method for the heat treatment of steel of the class which can be hardened by heating and quenching, which comprises heating the steel into its austenitizing range in a heating medium which is noncarburizing towards the steel for a time sufficient to heat the steel throughout, then transferring the hot steel to a molten salt bath held at a temperature in the range 700°-770° C. and containing at least 5 percent by weight of alkali metal cyanate calculated as  $N_xCNO$  and a remainder consisting essentially of alkali metal cyanide together with a salt selected from the group consisting of alkali metal carbonate and mixtures thereof with alkali metal chloride, and soaking the steel in said salt bath for at least 3 minutes and then rapidly cooling the steel.

10. 6. A method according to claim 1, wherein the said molten salt bath contains at least 10 percent by weight of alkali metal cyanate calculated as NaCNO.

15. 7. A method according to claim 1, wherein the step of heating the steel into its austenitizing range is carried out by immersing the steel in a neutral salt bath.

20. 8. A method according to claim 1, wherein the steel is a high-carbon steel and the step of heating the steel into its austenitizing range is carried out by immersing the steel in a molten salt bath containing alkali metal cyanide.

25. 9. A method according to claim 1, wherein the said molten salt bath held at a temperature in the range 700°-770° C. is restricted to the range 700°-750° C. the hot steel is immersed in this bath and is soaked therein for at least 5 minutes.

30

35

40

45

50

55

60

65

70

75